

## UNITED STATES PATENT OFFICE

2,267,261

## SMOKELESS POWDER

Elton E. Allison, Wharton, N. J., assignor to Hercules Powder Company, Wilmington, Del., a corporation of Delaware

No Drawing. Application November 6, 1940,  
Serial No. 364,480

4 Claims. (Cl. 52—5)

This invention relates to a method of preparing progressive burning smokeless powder and more particularly to an improved method of coating smokeless powder with a deterrent material, and to smokeless powder coated with a water soluble deterrent material.

It has been known to coat smokeless powder with a deterrent material in order to provide for a close control of the burning rate and to produce a high velocity of the projectile without excessively high breech pressures. Such coating materials desirably penetrate the powder grains more or less, so that as the powder burns, the successively exposed surfaces contain gradually less and less of the deterrent material, thus causing the combustion of the grains to proceed with increased speed.

Treatment of smokeless powder grains with a deterrent to render their combustion progressive, by methods heretofore known, while producing the desired results to a degree, has been open to a number of objections. For example, the use of a deterrent and powder grains alone requires long continued heat and tumbling to obtain uniform distribution of deterrent on the powder grain which may lead to explosion. The use of water with the deterrent and powder grains requires long treatment and renders uniform coating difficult on account of the water insolubility of many deterrents heretofore known. The use of a deterrent solvent, e. g., benzol, is open to the great risk of explosion of solvent vapors, their poisonous nature, and the economic necessity for recovery of the solvent. The use of prior known water soluble deterrents has furthermore not produced smokeless powder of high ballistic stability, i. e., the maintenance with age of the initial ballistics produced by the powder.

It is an object of this invention to produce a coated smokeless powder which overcomes the disadvantages of prior known powders.

It is a further object of this invention to produce a smokeless powder coated with a water soluble deterrent substance.

A still further object of this invention is to produce a smokeless powder coated with phthalide.

A further object of this invention is to produce a coated smokeless powder which has an improved hot storage ballistic stability.

Other objects will appear hereinafter.

The objects of my invention are accomplished by coating grains of smokeless powder with phthalide.

As an example for carrying out my invention

100 parts by weight of double base (20% N. G.) rifle powder granulated .045-.015 x 1/21 were placed in a sweetie or tumbling barrel and wet with 15 parts by weight of cold water. The wet powder was tumbled and heated to 75° C. and then 5 parts by weight of phthalide added. The mixture of powder, water and phthalide was agitated 30 minutes at 75° C. and 30 minutes at 85° C., removed from the barrel, dried, glazed and humidified. One portion of the powder was stored for 30 days at 50° C. and another portion for 30 days at normal atmospheric temperatures and then both portions rehumidified. The powder which had been stored hot was then tested in direct comparison with the powder which had been stored at normal temperatures. For the same charge of powder the hot storage sample produced 1,000 lbs./sq. in. higher pressure than the normal storage powder.

20 As a comparison with the above example, 100 parts by weight of double base (20% N. G.) rifle powder granulated .045-.015 x 1/21 were placed in a sweetie barrel and wet with 15 parts by weight of cold water. The wet powder was tumbled and heated to 75° C. and five parts by weight of diacetin added. The mixture of powder, water and diacetin was agitated 30 minutes at 75° C. and 30 minutes at 85° C., removed from the barrel, dried, glazed, and humidified. One portion of the powder was stored for 30 days at 50° C. and another portion for 30 days at normal atmospheric pressures and then both portions rehumidified. The powder which had been stored hot was then tested in direct comparison with the powder which had been stored at normal temperatures. For the same charge of powder the hot storage sample produced 9,100 lbs./sq. in. higher pressure than the normal storage powder.

30 The increased hot storage capacity of smokeless powder treated with water soluble phthalide as compared to the water soluble diacetin is apparent from the above examples. I am not at present prepared to give a sound theoretical explanation of the improved behavior of powder coated with phthalide as compared to powder coated with previously known water soluble deterrent agents. The most likely explanation is related to another physical property of the deterrent, i. e. its state of aggregation at the temperature of the ballistic stability storage test. The water soluble deterrents previously known were all liquids at both normal temperatures and at 50° C., the temperature of the hot storage ballistic stability test. Phthalide is a solid under

these conditions. It is my belief that poor ballistic stability is caused by mobility of deterrent molecules and that the molecules of deterrent substances which are in the liquid state under normal conditions will have greater mobility than those of materials which are solids under the same conditions. When a deterrent is applied to a smokeless powder grain, it penetrates into the powder grain surfaces more or less according to the temperature of application, the solvent or plasticizing power of the deterrent, and the state of aggregation of the deterrent. After the powder is dried, glazed, humidified and cooled to normal temperatures, this penetration due to deterrent mobility nearly ceases. It may continue at a very low rate at normal temperatures but if the powder is stored at somewhat higher temperatures the mobility and penetration tend to increase. Under these conditions the deterrent which is normally in the solid state of aggregation will give improved ballistic stability.

It is to be understood that single base as well as double base rifle powder may be treated in accordance with the teachings of this invention. The amount of phthalide added may be varied in accordance with the granulation of the powder and the deterrent effect desired. While 5% by weight of the weight of powder being coated was a satisfactory amount in the instance of the example given it is to be understood that I am

not limited to this proportion. Other granulations of powder may require from 1 to 10% by weight of phthalide to provide the desired deterrent action.

5 Where in this specification I refer to phthalide I mean the inner ester of o-hydroxy-methylbenzoic acid obtained by the reduction of phthalic anhydride or chloride with Zn and HCl and which has a melting point of 73° C., and a boiling point of 290° C.

10 My invention provides an improved smokeless powder having an increased hot storage ballistic stability, and one which is comparatively safely, economically and efficiently produced. This 15 powder may be used in the manufacture of cartridge ammunition.

What I claim and desire to protect by Letters Patent is:

1. A smokeless powder comprising smokeless 20 powder grains surface coated with phthalide.

2. A double base smokeless powder comprising smokeless powder grains surface coated with phthalide.

25 3. A single base smokeless powder comprising smokeless powder grains surface coated with phthalide.

4. A smokeless powder comprising smokeless 30 powder grains coated with phthalide in amount from about 1% to about 10% by weight of the powder.

ELTON R. ALLISON.